

## UNITED STATES PATENT OFFICE

2,672,445

## TRANSFORMER OILS

William T. Stewart, Berkeley, Charles D. Newnan,  
San Pablo, and Neal W. Furby, Berkeley, Calif.,  
assignors to California Research Corporation,  
San Francisco, Calif., a corporation of Delaware

No Drawing. Application April 29, 1950,  
Serial No. 159,142

12 Claims. (Cl. 252—47.2)

**1** This invention relates to the stabilization of lubricating oil compositions intended for use in the service of transformer oils, turbine oils and the like. More particularly, this invention pertains to the use of so-called synthetic lubricating oil compositions as transformer oils, wherein the anti-oxidation characteristics of the anti-oxidant present in the composition (e. g., selenium compounds) have been enhanced by the presence of hydroxy anthraquinone compounds (e. g., quinizarin).

This application is a continuation-in-part of the Stewart et al. application Serial No. 109,426 filed August 9, 1949.

For a number of years, it has been the general practice to use moderately treated mineral oils as transformer oils. However, these moderately treated oils gradually deteriorate in service. The effectiveness of transformer oils as insulating oils is materially reduced by oxidation products (i. e., the acid products) formed. These acid products also gradually attack the insulation on the wires of the transformer system, leaving the wires partially exposed to the oil, which oil then serves as a transmitter of current instead of an inhibitor of current. In the turbine oils the oxidation products (i. e., the acid sludges) corrode the bearings and other parts of the turbine system and clog the oil lines, etc.

It is a tremendous advantage in transformer, turbine, and like systems to use oils of sufficient oxidation stability to permit their use over long periods of time without being changed. Not only is it desirable to have transformer oils and the like highly resistant to oxidation, but it is also a desired feature of the transformer oils and the like that the viscosity index be high—that is, that only small changes in viscosity occur with large changes in temperature. Thus, in order to obtain oils of high viscosity index, it is advantageous in some instances to use synthetic oils which are prepared especially to resist changes in viscosity with changes in temperature.

In attempting to increase the oxidation stability of transformer and turbine oils, known oxidation inhibitors (such as the dialkyl selenides of Denison and Condit Patents Nos. 2,398,414 and 2,398,415) were incorporated therein, and, as expected, the resulting compounded oils were more resistant to oxidation than the base oils containing no inhibitors. However, it was not to be expected that the oxidation stability of the oil thus compounded with oxidation inhibitors could be increased still further by adding thereto an agent which by itself is not an oxidation inhibitor.

**2** It is an outstanding feature of this invention that the oxidation stability of lubricating oils compounded with oxidation inhibitors is materially increased by adding thereto an agent not known as an oxidation inhibitor which agent asserts synergistic effects in combination with the oxidation inhibitors of this invention.

It is a primary object of this invention to produce polyalkylene oxide lubricating oil compositions which are highly resistant to oxidation.

It is another object of this invention to incorporate in polyalkylene oxide oils containing oxidation inhibitors an agent exhibiting a marked synergistic effect on certain oxidation inhibitors.

It is a further object of this invention to produce transformer oils and the like which are more resistant to oxidation than those heretofore known.

These and other objects may be obtained from the disclosures and the claims noted hereinbelow.

It has been discovered that highly oxidation resistant polyalkylene oxide compositions of lubricating viscosity may be prepared by incorporating hydroxy anthraquinones in said compositions containing oxidation inhibitors, particularly, selenides.

Synthetic oils of the alkylene oxide type polymer which are used include those exemplified by the alkylene oxide polymers (e. g., propene oxide polymers) and derivatives, including alkylene oxide polymers prepared by polymerizing alkylene oxides, e. g., propylene oxide, in the presence of water or alcohol, e. g., ethyl alcohol, and esters of alkylene oxide type polymers, e. g., acetylated propene oxide polymers prepared by acetylating propene oxide polymers containing hydroxyl groups.

The hydroxy anthraquinones of this invention are anthraquinones containing at least one hydroxyl group on the ring, such as exemplified by 1-hydroxy anthraquinone, alizarin (1,2-dihydroxy-anthraquinone), quinizarin (1,4-dihydroxy anthraquinone), 1,5 - dihydroxyanthraquinone and 1,8-dihydroxy anthraquinone. It is preferred to use dihydroxy anthraquinones, particularly, quinizarin.

Oxidation inhibitors which are contemplated by this invention to be used in viscous oil compositions in combination with hydroxy anthraquinones include selenides. The particular selenides of the present invention may be represented by the formula:



wherein A is R<sub>1</sub>, Se—R<sub>2</sub>, M or a hydrogen atom; R, R<sub>1</sub> and R<sub>2</sub> are like or unlike substantially

hydrocarbonaceous organo groups connected to selenium through an aliphatic carbon atom, at least R, and preferably also R<sub>1</sub> and R<sub>2</sub>, contain at least 10 carbon atoms, preferably 12 to 30 carbon atoms, and M represents a cationic salt-forming radical, such as a metal atom. Thus, the selenides embrace di-organo mono- and di-selenides, selenomercaptans (organo hydroselenides) and selenomercaptides (metallo organo selenides). Preferred are the di-organo selenides (i. e., R'-Sen-R'', where n=1 or 2 and R' and R'' are like or unlike aliphatic radicals each of at least 10 carbon atoms); of these, the mono-selenides are ordinarily preferred.

Suitable organo groups, which are preferably hydrocarbon groups, include alkyl groups, such as decyl, lauryl, cetyl, etc., alkylated cycloaliphatic radicals, such as ethyl cyclohexyl, dimethyl cyclohexyl, etc., alkylated aralkyl radicals, such as cetylbenzyl, butylbenzyl, etc., and the aliphatic radicals derived from halogenated mixtures of hydrocarbons such as chlorinated naphtha, chlorinated kerosene, chlorinated paraffin wax, etc. The aliphatic groups may contain non-hydrocarbon substituents such as chlorine, bromine, hydroxyl and amino so long as their essentially hydrocarbon character remains substantially unchanged. Of these various types of organo groups, the alkyl radicals are preferred and of these, the dodecyl group is especially preferred.

The cationic salt-forming radical may be metals, such as sodium, calcium, barium, zinc, potassium, lithium, strontium, aluminum, lead, thallium, etc., or the ammonium radical. Preferably, the metals are the polyvalent metals, especially those of groups IIb, IV and VIII of the periodic table.

The following specific examples of selenides will further illustrate the selenium compounds of the present invention: dialkyl selenides, such as octyl decyl monoselenide, dilauryl monoselenide, dieicosyl monoselenide, dialkyl diselenides, such as didecyl diselenide, didodecyl diselenide (dilauryl diselenide), diheptadecyl diselenide, dieicosyl diselenide, selenomercaptans, such as lauryl selenomercaptan, cetyl selenomercaptan, octadecyl selenomercaptan, paraffin wax selenomercaptan, etc., and the corresponding sodium, calcium, barium, zinc, cadmium and lead salts of such selenomercaptans.

The oxidation inhibitors (i. e., the organic selenium compounds) which are present in the lubricating oil composition may be present in amounts from about 0.0001% to about 5% by weight of the final composition, that is, an amount sufficient to increase the resistance of the lubricating oil composition to oxidation. It is preferred to use from about 0.1% to about 2.0%.

The hydroxy anthraquinones of this invention (e. g., quinizarin) may be present in the final mineral oil composition in amounts from about 0.0001% to about 1.0% by weight of the final composition. It is preferred to use an amount sufficient to enhance the oxidation-inhibiting characteristics of the organic selenium compound, preferably from about 0.02% to about 0.1%.

The organic selenium compound can be replaced in part by alkylated phenol oxidation inhibitors, such as 2,6-di-tertiary butyl-4-methyl phenol, to procure a long life for the compounded oil. This is desirable since it provides a way of cutting down the amount of expensive selenide without reducing the long life as obtainable

with selenides alone. Thus, a hydroxy anthraquinone (e. g., quinizarin) may be added to a lubricating oil containing an alkylated phenol oxidation inhibitor (e. g., 2,6-di-tertiary butyl-4-methyl phenol) and a selenide oxidation inhibitor (e. g., dilauryl monoselenide) to obtain a long life for the compounded oil.

A remarkable feature of this invention is the wholly unexpected, greatly enhanced synergistic effects which are obtained between lubricating oil oxidation inhibitors (e. g., organic selenium compounds) and the hydroxy anthraquinones (e. g., quinizarin). Nowhere would any one expect to find such synergistic effects as disclosed herein by the addition of a hydroxy anthraquinone as a secondary agent to a lubricating oil composition containing additives which are known to inhibit oxidation, particularly to find its anti-oxidation properties enhanced so tremendously by the addition of a secondary agent which in itself has relatively no effect in inhibiting oxidation in a lubricating oil. Obviously, it is not merely an additive effect which is obtained between the combinations of the known oxidation inhibitor in the lubricating oil and the hydroxy anthraquinones because the hydroxy anthraquinones in themselves are practically ineffective in inhibiting the oxidation in the lubricating oil composition.

In the table hereinbelow, data are presented to show the synergistic effects obtained by testing the compositions of additives in a polyalkylene oxide lubricating oil under severe conditions. In order to test effectively the compositions of this invention, a more drastic test was devised than is normally used in evaluating transformer oils and the like. This test has been called the California Research Transformer Oil Stability Test. The test is run as follows:

A 300 gram sample to be tested is placed in a glass tube which is set in an oil bath at 250° F. Oxidation catalysts, i. e., 112½ square centimeters of medium silicon transformer iron (such as USS Trancor 72) and 450 square centimeters of No. 14 gauge ASTM electrolytic copper wire are inserted in the tube. Oxygen is bubbled through the test sample at the rate of 3 liters per hour until the test sample has an acid number of 1.0 (milligrams of KOH per gram sample of oil). The number of hours required for the sample to show an acid number of 1.0 is known as the "Test Life" of the sample.

The data presented in Table I will serve to illustrate the nature of the results that were obtained in accordance with the present invention. The base oil used in obtaining the data of Table I is described as an iso-octyl alcohol-initiated polypropene oxide acetate, having a viscosity of 88 SSU at 100° F. The following equations and Example I exemplify the manner in which the iso-octyl alcohol-initiated polypropene oxide acetate was obtained:



wherein R and R<sub>1</sub> represent hydrocarbon radicals, and n refers to the number of alkylene oxide units present.

## EXAMPLE I

A mixture of 0.75 part by weight of metallic sodium and 32.1 parts by weight of 2-ethyl hexanol was heated with agitation to 200-220° F. while sweeping out the hydrogen evolved with nitrogen. After hydrogen evolution ceased, the vessel and contents were heated to 240° F. Propene oxide having a water content of less than 0.1% was added until the pressure in the vessel was 40 p. s. i. (pounds per square inch). As the polymerization progressed, additional propene oxide was added to maintain the pressure at 40 p. s. i. while holding the temperature at 240° F. until 115 parts of propene oxide had been added. Thereafter the reaction mixture was stirred for an additional hour. 15 parts by weight of acetic anhydride were then added and the reaction mixture was heated at 300° F. for 4 hours, after which time the impurities and unreacted ingredients were removed by stripping at a pressure of about 25 mm. of mercury with a pot temperature of about 300° F. The residue was then filtered.

In the specific base oil used in the examples of Table I, the mol ratio of alcohol to propene oxide was 1 to 8. This synthetic oil is also termed a polypropene glycol octyl ether acetate.

Table I

| Oil                                              | "Test Life"<br>(Hrs.) |
|--------------------------------------------------|-----------------------|
| Base Oil.....                                    | Less than 20.         |
| Base Oil+0.05% Quinizarin.....                   | Do.                   |
| Base Oil+2.0% Dilauryl Selenide.....             | 250.                  |
| Base Oil+2.0% Dilauryl Selenide+0.05% Quinizarin | 570.                  |

From the above data, it is readily seen that the combination of an alkyl selenide and a hydroxy anthraquinone is more effective by far in inhibiting oxidation in a synthetic oil than is either one of the compounds by itself.

The polyalkylene oxide lubricating oil compositions of the present invention have their present field of chief utility in transformer oils and in turbine oils. However, the compositions of this invention may be used in high-temperature gas turbines, hydraulic systems, ice machines, instruments, etc.

The hydroxy anthraquinones may also be used in oils containing other groups of additives in addition to anti-oxidants. For example, in addition to the above-noted compounds, these lubricating oils may contain other agents, such as pour point depressants, oiliness agents, extreme pressure agents, blooming agents, compounds for enhancing the viscosity index of the synthetic oils, grease-forming agents, peptizing agents, etc.

As used herein, the terms "substantially hydrocarbonaceous" and "essentially hydrocarbon" refer to groups which are composed almost entirely of only hydrogen and carbon atoms. It is not intended that the hydrogen and carbon atoms are the only atoms present. The terms embrace groups which are composed almost entirely of hydrogen and carbon atoms and the derivatives of these groups. That is, in addition to the hydrogen and carbon atoms, the groups may contain chlorine, bromine, hydroxyl, amino groups, etc., so long as there are sufficient hydrogen and carbon atoms present to retain the hydrocarbon character of the groups.

We claim:

1. A lubricating oil composition consisting essentially of a major portion of a low molecular

weight alkylene oxide liquid polymer of lubricating viscosity, which polymer is substantially free from groups normally reactive with selenides and dihydroxyanthraquinones, and a small amount, sufficient to increase the resistance of the lubricating oil to oxidation, of a selenide having at least one aliphatic group of at least 10 carbon atoms attached to the selenium atom, to which lubricating oil composition is further added a synergist for the selenide, said synergist being a dihydroxyanthraquinone which is present in the lubricating oil composition in an amount from about 0.0001% to about 1.0%, by weight.

2. A lubricating oil composition consisting essentially of a major portion of a low molecular weight alkylene oxide liquid polymer of lubricating viscosity, which polymer is substantially free from groups normally reactive with selenides and dihydroxyanthraquinones, and a small amount, sufficient to increase the resistance of the lubricating oil to oxidation, of a selenide represented by the formula



wherein R and R<sub>1</sub> are aliphatic groups containing at least 10 carbon atoms, to which lubricating oil composition is further added a synergist for the selenide, said synergist being a dihydroxyanthraquinone which is present in the lubricating oil composition in an amount from about 0.0001% to about 1.0%, by weight.

3. A lubricating oil composition consisting of a major proportion of an esterified low molecular weight alkylene oxide liquid polymer of lubricating viscosity, which polymer is substantially free from groups normally reactive with selenides and dihydroxyanthraquinones, and from about 0.0001% to about 5%, by weight, of a selenide having at least one aliphatic group of at least 10 carbon atoms attached to the selenium atom, to which lubricating hydrocarbon oil composition is further added a synergist for the selenide, said synergist being a dihydroxyanthraquinone which is present in the lubricating oil composition in an amount from about 0.0001% to about 1.0%, by weight.

4. A lubricating oil composition consisting of a major proportion of a low molecular weight alkylene oxide liquid polymer of lubricating viscosity, which polymer is substantially free from groups normally reactive with selenides and hydroxyanthraquinones, and from about 0.1% to about 2.0%, by weight, of a selenide having at least one aliphatic group of at least 10 carbon atoms attached to the selenium, to which lubricating oil composition is added a synergist for the selenide, said synergist being a dihydroxyanthraquinone, and being present in the lubricating oil composition in an amount from about 0.02% to about 0.1%, by weight.

5. A lubricating oil composition consisting essentially of a major portion of a low molecular weight alkylene oxide liquid polymer of lubricating viscosity, which polymer is substantially free from groups normally reactive with selenides and dihydroxyanthraquinones, and a small amount, sufficient to increase the resistance of the lubricating oil to oxidation, of a selenide represented by the formula



wherein R and R<sub>1</sub> are aliphatic groups containing at least 10 carbon atoms, to which lubricating oil composition is further added a synergist for the selenide, said synergist being a dihydroxyan-

thraquinone which is present in the lubricating oil composition in an amount from about 0.0001% to about 1.0%, by weight.

6. A lubricating oil composition consisting essentially of a major portion of a low molecular weight alkylene oxide liquid polymer of lubricating viscosity, which polymer is substantially free from groups normally reactive with selenides and dihydroxyanthraquinones, and a small amount, sufficient to increase the resistance of the lubricating oil to oxidation, of a selenide represented by the formula



wherein R is an aliphatic group containing at least 10 carbon atoms and M is a cationic salt-forming radical, to which lubricating oil composition is further added a synergist for the selenide, said synergist being a dihydroxyanthraquinone which is present in the lubricating oil composition in an amount from about 0.0001% to about 1.0%, by weight.

7. A low molecular weight alkylene oxide liquid polymer of lubricating viscosity, which polymer is substantially free from groups normally reactive with selenides and dihydroxyanthraquinones, to which is added a small amount, sufficient to increase the resistance of said alkylene oxide liquid polymer to oxidation, of a selenide having at least one aliphatic group of at least 10 carbon atoms attached to the selenium atom, to which composition is further added a synergist for the selenide, said synergist being a dihydroxy-

anthraquinone which is present in the alkylene oxide liquid polymer lubricating composition in an amount from about 0.0001% to about 1.0%, by weight.

8. The lubricating oil composition of claim 4, wherein the low molecular weight alkylene oxide liquid polymer of lubricating viscosity is an alcohol initiated and esterified polymerization product of low molecular weight alkylene oxide.

9. The lubricating oil composition of claim 4, wherein the low molecular weight alkylene oxide liquid polymer of lubricating viscosity is an octyl alcohol initiated polypropene oxide acetate.

10. The lubricating oil composition of claim 4, wherein the selenide is a dialkyl monoselenide.

11. The lubricating oil composition of claim 4, wherein the selenide is dilauryl monoselenide.

12. The lubricating oil composition of claim 4, wherein the hydroxy anthraquinone is quinizarin.

WILLIAM T. STEWART.  
CHARLES D. NEWNAN.  
NEAL W. FURBY.

25 References Cited in the file of this patent  
UNITED STATES PATENTS

| Number    | Name                 | Date           |
|-----------|----------------------|----------------|
| 2,016,648 | Orelup               | Oct. 8, 1935   |
| 2,214,443 | Varteressian         | Sept. 10, 1940 |
| 2,398,415 | Denison, Jr., et al. | Apr. 16, 1946  |
| 2,434,978 | Zisman               | Jan. 27, 1948  |
| 2,497,097 | Roberts              | Feb. 14, 1950  |